

Patented Dec. 12, 1922.

1,438,431

# UNITED STATES PATENT OFFICE.

WILHELM ESCHBACH, OF TROISDORF, GERMANY.

## BLASTING DETONATOR.

No Drawing.

Application filed February 3, 1921. Serial No. 442,279

To all whom it may concern:

Be it known that I, WILHELM ESCHBACH, citizen of Germany, and resident of Troisdorf, Germany, have invented certain new and useful Improvements in or Relating to Blasting Detonators, of which the following is a specification.

For blasting detonators, the filling of which consists of fulminate of mercury or of trinitrotoluene or tetrannitromethylaniline with a top charge of fulminate of mercury, shells have hitherto been used which are made of copper, brass, zinc or similar metals. Shells of this kind, particularly zinc and brass shells, have however the disadvantage that, when they are clipped on to the quick-match by means of the clamping tongs they are easily split with the result that firstly they are liable to explode prematurely and secondly it is impossible to make a tight joint with the quick-match. For this reason misfires very easily occur in bore holes which contain water. Even the copper shells possess this disadvantage, although in a lesser degree, as the metal due to its being repeatedly worked is too brittle.

The use of aluminium in place of copper or brass for the manufacture of blasting detonators shells has hitherto not been suggested as this metal is completely destroyed in a short time by the fulminate of mercury.

It has now been found possible to manufacture a blasting detonator, the shell of which consists of aluminium and the charge thereof of lead azide, lead azide mixtures or similar materials, which behave inertly towards this metal and which is free from the above mentioned disadvantages. Splitting of the metal when clamping the shell on to the quick-match is precluded, on account of the malleability of the aluminium, whereby premature explosion is avoided and a tight joint secured with the quick-match thus preventing the penetration of any water which there may be in the bore hole into the percussion caps.

As it is not necessary to use an inner cap for these new blasting detonators, the advantage of a greater surface of ignition is secured in addition to the saving in metal.

With regard to storage in damp places, experiments which have been carried out for several years have proved that aluminium caps loaded, for example, in their lower part with tetrannitromethylaniline and with

a top charge of lead azide or mixtures of lead azide or the like detonating composition which are inert towards this metal showed no oxidation phenomena whatsoever. Even 60 caps stored in the outlet current of a Westphalian mine for a long time had neither become decomposed nor oxidized and bore no signs of this kind. When fired at a leaden plate a normal image was also obtained. 65 This fact, that is to say the disinclination of aluminium to oxidize of itself, is therefore of great importance for the manufacture of blasting detonators.

The easy malleability of aluminium is obviated by the drawing process which the shell has to go through from the strip up to its completion. The shell thus acquires a sufficient degree of hardness which protects it from distortion. By this means also any 70 loosening or crumbling of the loading is prevented especially if the loading contains an admixture of some adhesive substance and is forced in under high pressure. The dead pressing of the loading which very easily 75 occurs with fulminate of mercury is in this case impossible.

The technical advance of the present invention is therefore to be found in the fact that in place of copper, brass or zinc aluminium can be used for the manufacture of shells for blasting detonators. Furthermore these aluminium caps have in comparison with copper caps with exactly the same charge a much greater co-efficient of initiation. Experiments with the Trauzl leaden block as well as transmission firings have 80 shown these caps to be free from objection. A further proof of the superiority of these caps compared with copper ones is that the 85 aluminium caps when fired at the leaden plate show a considerably finer radiation.

Having now particularly described and ascertained the nature of my said invention and in what manner the same is to be performed, I declare that what I claim is:—

In the manufacture of blasting detonators the use of an aluminium shell with a loading of lead azide or mixtures of lead azide and similar detonating compositions which are 90 inert towards said metal and which can be easily clipped on to the quick-match by the clamping tongs.

Signed at Treisdorf in the State of Germany this 15<sup>th</sup> day of December 1920,

WILH. ESCHBACH.